

Oct. 31, 1933.

J. D. DOHERTY

1,932,815

## TREATED COKE AND PROCESS OF TREATING THE SAME

Filed Feb. 28, 1931



INVENTOR.  
Joseph D. Doherty.  
BY Jessie R. Langley  
ATTORNEY.

## UNITED STATES PATENT OFFICE

1,932,815

TREATED COKE AND PROCESS OF  
TREATING THE SAMEJoseph D. Doherty, Pittsburgh, Pa., assignor to  
The Koppers Company of Delaware, a corpora-  
tion of Delaware

Application February 28, 1931. Serial No. 519,103

10 Claims. (Cl. 44—6)

My invention relates to treated coke and process of treating the same and particularly to processes for marking coke for identification and for rendering the coke substantially dustless.

5 My invention is related to, and is an improvement upon, that described and claimed in the application of Gilbert V. McGurl, Serial No. 434-176, filed March 7, 1930.

In accordance with the present invention, I 10 provide dyed pulp of such character as that ordinarily employed in the manufacture of paper and which may be of any desired color. The pulp is in such fluid state and is so mixed with a solution of a deliquescent salt, such as calcium chloride or magnesium chloride, that the mixture may 15 be readily applied by means of fluid pressure to a moving stream of coke. The solution containing the pulp may be supplied in such quantities as to be applied to substantially all of the 20 pieces of coke whereby the latter are rendered distinctive in appearance and receive a sufficient quantity of the solution to render the coke substantially dustless.

In preparing a suitable mixture for treating 25 the coke, fibrous pulp, such as may be employed in connection with the manufacture of paper in paper mills, is supplied to a suitable beater after the latter is partially filled with water. The weighed amount of pulp is sufficient to make 2.5 30 to 3% of stock. The pulp is then disintegrated in the water and the correct amount of dye in solution is added.

Many fast dyes have slight affinity for pulp and it is necessary in many instances to employ 35 materials for fixing the dye on the pulp fibres. It has been found that rosin size and an alum or other suitable chemical, for example, aluminium sulphate ( $Al_2(SO_4)_3 \cdot 18H_2O$ ) are satisfactory for this purpose. When used, the rosin 40 size is preferably added immediately after the dye and the alum is added shortly before the completion of the beating process.

When, however, calcium chloride solution is 45 employed, as in the process of my invention, it serves to fix the dye on the fibres of the pulp and the addition of rosin size and an alum may be dispensed with, if desired.

Tests have shown that the following mixture 50 provides a treating material with very satisfactory characteristics as to distinctive color and its durability and as to rendering the coke substantially dustless:

Pulp..... 200 pounds sulphite screenings  
55 Water..... 390 gallons

Dye..... 2 pounds Solantine red 8 BLNP  
Sizing..... 4 pounds rosin size  
(If desired)..... 5 pounds alum  
Deliquescent salt..... 545 gallons 33%  $CaCl_2$  solution

60 The following is an example of a procedure of preparing such a mixture from said quantities. Into a beater capable of holding 200 pounds of air-dry pulp at 5-6% consistency (percent air-dry pulp in mix) run 390 gallons of water and then add 200 pounds of air-dry pulp. After the pieces are broken up sufficiently 3 gallons of dye solution containing 2 pounds Solantine red 8 BLNP dye are added and treatment in the beater continued for two hours. (Size and alum to be 65 added if desired.) The treated pulp is then dumped into an agitator tank and followed by 545 gallons of 33%  $CaCl_2$ . This produces a mixture comprising the suspension of colored pulp 70 which equals about 40-50 percent of the total mixture and the solution of calcium chloride 75 which equals about 60-50 percent of the total mixture.

2.4 gallons of this mixture contains approximately 0.5 pounds of pulp and five pounds of  $CaCl_2$ , which quantities are sufficient for trademarking and rendering substantially dustless 80 one ton of coke.

It will be understood that the concentrations 85 of pulp and calcium chloride and the quantity of mixture sprayed can be varied between rather wide limits. Dry calcium chloride may be added to dyed pulp or, if necessary, pulp can be dyed in a calcium chloride solution. However, when adding commercial calcium chloride to certain 90 unsized dyed pulps, the alkalinity must, in some cases, be adjusted as it affects the color of the pulp, when the solution is strongly alkaline. When the pulp is sized, however, the dye is not 95 adversely affected.

Instead of sulphite screenings, it is possible to use any fibrous or semi-fibrous pulp, such, for example, as cornstalk pulp, groundwood pulp, groundwood screenings, old newspapers, bleached sulphite, unbleached sulphite or soda pulp. Certain of these alternative materials or mixtures of two or more of them may be used satisfactorily but in some cases slightly more dye is required for the same depth of color and the resulting material does not retain its depth of color for the 105 same period. Bleached sulphite, unbleached sulphite and soda pulp may be substituted very satisfactorily for sulphite screenings, but their cost is somewhat higher.

The preferred dye employed, which is known 110

commercially as Solantine red 8 BLNP, may, if desired, be replaced by any suitable dye or pigment to obtain various shades and colors. The dye employed in the preferred mixture, however, has been found to be very satisfactory by reason of its fast and brilliant red color.

Upon the completion of the process of beating the pulp and adding the other ingredients, the mixture is transferred to a tank for storage. 10 Agitation is necessary to maintain a uniform mixture.

The prepared mixture may then be pumped or fed by gravity from the agitator tank to the sprays or other devices for applying the mixture to the coke. Any satisfactory type of spray may be used that will secure proper supply and distribution of the dyed pulp mixture. For example, the apparatus shown in the accompanying drawing may be employed.

20 In the drawing,

Figure 1 is an elevational view illustrating apparatus for loading and treating coke;

Fig. 2 is an enlarged detail view, partially in elevation and partially in vertical section, of a spray device for practicing my invention;

25 Fig. 3 is a plan view of a deflector of the device of Fig. 2; and

Figs. 4 and 5 are, respectively, top plan and side elevational views of a spray device of modified form.

30 In treating coke in accordance with my invention, coke may be supplied from a storage bin 1 to a conveyor belt 2, by means of which it is conveyed to a truck 3 or other container to be loaded. A pipe 4, which may be connected to any suitable storage device for the treating mixture, supplies the latter to a spray device 5 having a deflector 6 for directing the mixture downwardly in a spray of fan shape. The mixture may be forced through an orifice 7 in the end of the pipe 4 by means of liquid pressure, as by a pump. The mixture comprising the dyed pulp is indicated at 8.

35 As shown in Fig. 2, the operation of the spray device 5 may be controlled by means of a valve 9 having, for example, bevel gear mechanism 10 and a sprocket wheel 11 and a chain 12 therefor for conveniently adjusting the position of the valve 9.

40 In case it is desired to spray the solution over a band of moving coke, as in a chute, the spray device 14 shown in Figs. 4 and 5 may be used. It is provided with a whirling chamber 15 and an outlet or nozzle 16 from which the material 45 diverges in the form of a cone.

45 By suitably regulating the pressure and thereby the quantity of mixture that is applied to the coke, the latter may be marked to any desired degree and the coke may be supplied with a desired amount of calcium chloride solution for rendering the coke dustless. Coke thus treated will have a distinct appearance that will readily identify it from coke marked by any other material. It will retain its means of identification since the pulp readily conforms to the porous surface of the coke and adheres thereto, where it will remain for long periods, regardless of weather conditions.

50 The pulp will also retain its brilliance of color for considerable periods by reason of the dye being fixed on the fibres of the pulp and by reason, also, of the fact that the pulp remains slightly moist because of the presence of the deliquescent salt. Furthermore, the surface coating of the calcium chloride solution on the coke

causes the latter to remain moist under substantially all conditions and thereby reduces the tendency of the coke to emit small particles.

55 The coke may be treated for marking and for rendering it dustless at any desired stage in its handling after being quenched but preferably as it is being loaded for shipment or for delivery to the consumer. The coke should be free falling or tumbling, as in a chute, when the mixture is applied.

60 Coke marked with the materials and in the manner above described possesses a number of advantageous features. The marking material is of fast color and it will retain its appearance for relatively long periods of time. The marking material is firmly secured to the coke by reason of its conforming to the rough cellular structure of the latter. The marking material is combustible and contains very little ash. The marking material has no odor and coke marked as described above has a pleasing appearance.

65 The presence of calcium chloride in the treating mixture causes the latter to have a much lower freezing point and, consequently, the process may be practiced in relatively cold weather without freezing of the pulp suspension in the pipes. For the same reason, freezing of treated coke in cars and bins is also prevented.

70 The use of calcium chloride solution permits the omission of sizing for fixing dye on the fibres, if desired, and the color is deepened and its appearance is the more brilliant by reason of the pulp being in a more moist condition. The fastness of the color to light is also increased.

75 It will be appreciated that the proportions of the various ingredients of the treating mixture may be varied within reasonable limits and the quantity of the treating mixture may be varied in accordance with the results that are to be secured.

80 The foregoing and other advantages will be apparent to those skilled in the art relating to the treatment of coke.

I claim as my invention:

1. The process of treating coke which comprises applying to the outer surface thereof a mass of colored pulp and calcium chloride solution.

2. Coke having on the outer surface thereof a mass of colored pulp and calcium chloride solution.

3. The process of treating coke which comprises applying thereto dyed fibrous pulp and deliquescent material for fixing dye on the fibres of said pulp and for maintaining said pulp and the surface of said coke in moist condition.

4. Coke having applied thereto dyed fibrous pulp and deliquescent material for fixing dye on the fibres of said pulp and for maintaining said pulp and the surface of said coke in moist condition.

5. The process of treating coke which comprises applying thereto a composition comprising a mixture of about forty to fifty parts of a suspension of colored fibrous pulp and about sixty to fifty parts of a solution of calcium chloride.

6. The process of treating coke which comprises applying thereto a composition comprising a mixture of about forty to fifty parts of a suspension of colored fibrous pulp and about sixty to fifty parts of a solution of approximately 33% calcium chloride.

7. The process of treating coke which comprises applying to each ton thereof between 2.4 to three gallons of a composition containing col-

- ored fibrous pulp suspension and calcium chloride solution.
8. The process of treating coke which comprises applying to each ton thereof approximately 5 2.5 gallons of a composition comprising a mixture of about forty-five parts of a suspension of dyed fibrous pulp and about fifty-five parts of a solution of 33% calcium chloride for marking said coke to render it distinctive for identification and 10 for rendering it substantially dustless.
9. The process of treating solid fuel of the lump character of coke which comprises apply-
- ing to the outer surface thereof a quantity of colored fibrous pulp and a solution of a deliquescent salt for both fixing the color on the fibres of said pulp and for rendering the coke substantially dustless.
10. The process of treating coke which comprises applying thereto a composition of dyed fibrous pulp suspension and calcium chloride solution in which the ratio of pulp to calcium chloride is about one to ten.

JOSEPH D. DOHERTY.

|    |     |
|----|-----|
| 15 | 90  |
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |